

Patented Aug. 10, 1926.

1,595,872

# UNITED STATES PATENT OFFICE.

ALLEN ROGERS AND BISHAN NARIAN MATHUR, OF BROOKLYN, NEW YORK.

## OIL TANNING.

No Drawing.

Application filed August 31, 1925. Serial No. 53,719.

This invention relates to oil tanning; and it comprises a method of converting skins or hides into leather of the character of chamois, crown, etc., wherein the skin is milled and otherwise treated with a soapy composition of pasty nature containing water and alkali-containing saponified products derived from oils, this composition being most advantageously made from marine animal oil; all as more fully hereinafter set forth and as claimed.

In the usual routine of operation, in making leather from skins by the oil tanning or samian process skins are placed in stocks, oil added and the skins milled, usually for about four hours. They are then piled down and again milled and so on until the oil is well absorbed when the skins are placed in a warm room to dry out the water and complete the tanning, being thereafter pressed to remove the excess of oil, washed in a sodium carbonate solution, dried, staked and buffed. The whole operation takes about ten days.

It is the object of the present invention to provide a method of producing this class of leather, economizing time and giving a better product. To this end, instead of using oil, as in the ordinary method of operation, we employ a saponified product derived from such oils with the aid of alkali. All of these oils contain glycerids of unsaturated fatty acids of oily nature whose exact character is not very well known. Probably acids of the oleic series  $C_{18}H_{34}O_2$  and  $C_{17}H_{32}O_2$  are always present although oils from different sources are technically different. While other oils may be used we find it most advantageous for the present purposes to employ marine animal oils of the type of cod oil, shark liver oil and seal oil and make soaps therefrom in a special way. While we do not wish to limit ourselves to any theory it is believed that in this operation of making soap the unsaturated portion of the molecular group of the fatty acid in the oil readily becomes hydroxylated; giving eventually bodies which unite with the hide substance. And apparently upon the particular structure of the unsaturated acids depends much of the final result. At all events while tanning may be obtained in greater or less degree by the use of soapy products made from oils from other sources, marine animal oils give the best results. Soaps suitable for

our purpose may be made by heating marine animal oils, or mixtures of the same, with strong caustic soda solution to a temperature of about  $170^{\circ}$  F; the amount of the soda 60 solution being somewhat less than that necessary to saponify all the oil. Potash may be used in lieu of soda but is not better. An alkaline composition is, not desired in the present process and it is safer to leave 65 the soap with some unchanged oil to avoid occurrence of any excess of alkali. A  $20^{\circ}$  Baumé caustic soda solution is a desirable strength. Under the influence of heat and in the presence of the water of the mixture, 70 the unsaturated groups of the fatty acids of the oil apparently become eventually hydroxylated; giving solutions having a strong affinity for the amino substances of hide. Free acids made from these soaps have a 75 tanning action but are not so efficient as the soaps and are not as convenient to use.

The pasty water-containing mass of soaps made in the way just described, or in any other suitable manner, without removal of 80 the water, is used in oil tanning in lieu of the customary oil, the physical operations performed and the succession of steps being otherwise essentially the same.

Using the soapy material it is only necessary to mill the skins therewith for three or four hours, hang up to dry, or pack down over night, mill for two hours the next day and hang up to dry in a warm room. Under some circumstances in one stage of operation we may use some oil in addition to the soaps. When the skins are dried tannage is complete and nothing more is needed than the washing and drying to give a finished leather. The process works quicker at 85 around  $100^{\circ}$  F. than at ordinary temperature; but drying at room temperature may be used. Producing leather in this manner the whole operation can be completed in three or four days, which includes washing, 90 staking and buffing.

A charge of suitable soapy material for the present process may be made by placing into a soap crutcher or kettle 60 pounds of seal oil, shark liver or cod liver oil and heating to  $170^{\circ}$  F. To the warm oil is added a cool solution of 6 pounds of commercial caustic soda in 35 pounds of water. The mixture of oil and lye is stirred until smooth and is then dumped into a container for 105 cooling. When cooled the product is a smooth paste of the consistency of lard; this

paste containing the original water, some glycerine, soaps of the unsaturated and saturated acids of the oil and a little unchanged oil. The amount of soda used is about sufficient to give a 75 per cent saponification; that is to leave about 25 per cent of unchanged oil. The foregoing is given merely as a good way of producing desirable material for the present purposes. Other ratios 10 of oil and caustic soda may be used; and the temperature varied, but on the whole we find that a 75 per cent saponification gives the best result. While other oils may be employed, they do not give as good results. 13 Where other oils, such as menhaden, whale or even linseed or olive oils are to be used, it is better to use them in admixture with at least some of the marine animal oils specified. Of the marine animal oils we find that 20 on the whole the best results are given by cod liver, shark liver oils and seal oils.

In using a composition made as described, the skins or hides are milled with it in stocks or mills for about two hours, using about 25 half a gallon of the paste for each dozen average skins. After milling for two hours one-fourth gallon or more of the paste is introduced and milling resumed, usually for about two hours. The skins may then be 30 placed in piles or hung over night in a moderately warm room and the next day milled again for two hours, after which one-fourth gallon or more of the paste is added with the resumption of milling for two 35 hours more or until the compound is well absorbed. When the material is sufficiently worked into the skins they are hung up in a warm loft and allowed to dry slowly, the temperature of the drying room being, advantageously, between 110 and 120° F. A 40 closed room gives the best results. After drying the skins are washed in warm water, say 100° F. The water may contain a small amount of soda ash. After washing the 45 skins are again dried, milled to soften them and finally buffed.

The foregoing directions are, of course, merely given as exemplificatory. The amount of compound required of course 50 varies with the size of the skin. As a rule, however, we use about 50 per cent of compound on the pickled weight of the hides or skins. The described method may be combined with the usual methods of oil tanning. 55 For example in a modified form of our invention, the soapy compound is used for a preliminary treatment and the hides or skins are then treated with straight oil or a mixture of compound and oil. In so doing the 60 weakening effect of straight oil is obviated and more stretch is secured.

Leather produced in this manner does not get hard when used for washing automobiles and has more strength and body than the 65 usual chamois skin. It can be used for many

other purposes and we regard the present process as applicable in the manufacture of chamois, crown leather, buff leather, glove leather, etc. It can also be applied with advantage in the treatment of furs during the 70 leathering operation.

While not desiring to limit ourselves to any theory in the matter it is our present impression that unsaturated fatty acids, and particularly those occurring in marine animal oils become hydroxylated at the point of "double bond"; the point at which there is a double union between carbon atoms. Such a double union characterizes these unsaturated acids. And it is our present belief that the hydroxylated group enters into chemical union with amino groups in the hide substance. Certainly in the present process there is not an oxidation of the type which is supposed to characterize the reactions in the usual processes of oil tannage. 80

However, as stated, we do not limit ourselves to any theory but desire to claim merely the method of producing the results we secure; viz, tanning of skins and furs with a soapy paste made by reaction of caustic alkali on oils; and particularly marine animal oils. 90

What we claim is:—

1. A process of producing so-called oil 95 tannage of furs and skins wherein tanning is effected with an alkali-containing soapy composition of pasty nature containing an excess of oil and made from marine animal oils. 100

2. A process of producing so-called oil tannage of furs and skins wherein tanning is effected by water-containing soapy material, such soapy material containing alkali saponified products of marine animal oils 105 and unchanged oil and being of pasty nature. 110

3. In the manufacture of oil tanned furs, skins and hides, the process which comprises saponifying marine animal oils with an 115 amount of caustic alkali solution sufficient to saponify part but not all of the oil and working the pasty product thereby produced into the material to be tanned.

4. A process of producing so-called oil 115 tannage of furs and skins wherein a preliminary tanning is effected in a soapy product made from marine animal oil, and containing an excess of oil and completing the tanning by oil tanning. 120

5. A process of producing so-called oil tannage of furs and skins wherein tanning is effected with a pasty mixture of oil and of soap made from a marine animal oil and alkali. 125

In testimony whereof, we have hereunto affixed our signatures, this 29 day of August, 1925.

ALLEN ROGERS.  
BISHAN NARAIN MATHUR.